



US008691740B2

(12) **United States Patent**  
**Vickerman et al.**

(10) **Patent No.:** **US 8,691,740 B2**  
(45) **Date of Patent:** **Apr. 8, 2014**

(54) **OXALIC ACID BIS-AMIDES OR  
AMIDE-ESTER AS FRICTION MODIFIERS IN  
LUBRICANTS**

(75) Inventors: **Richard J. Vickerman**, Stow, OH (US);  
**Daniel J. Saccamano**, Sheffield (GB)

(73) Assignee: **The Lubrizol Corporation**, Wickliffe,  
OH (US)

(\*) Notice: Subject to any disclaimer, the term of this  
patent is extended or adjusted under 35  
U.S.C. 154(b) by 200 days.

(21) Appl. No.: **13/201,671**

(22) PCT Filed: **Feb. 11, 2010**

(86) PCT No.: **PCT/US2010/023855**

§ 371 (c)(1),  
(2), (4) Date: **Oct. 11, 2011**

(87) PCT Pub. No.: **WO2010/096321**

PCT Pub. Date: **Aug. 26, 2010**

(65) **Prior Publication Data**

US 2012/0021958 A1 Jan. 26, 2012

**Related U.S. Application Data**

(60) Provisional application No. 61/153,414, filed on Feb.  
18, 2009.

(51) **Int. Cl.**  
**C10M 133/16** (2006.01)

(52) **U.S. Cl.**  
USPC ..... **508/500**; 508/551; 508/554

(58) **Field of Classification Search**  
USPC ..... 508/500, 551, 554, 555  
See application file for complete search history.

(56)

**References Cited**

**U.S. PATENT DOCUMENTS**

|                 |   |         |                       |         |
|-----------------|---|---------|-----------------------|---------|
| 3,214,460 A     | * | 10/1965 | McGee et al. ....     | 560/155 |
| 3,251,853 A     |   | 5/1966  | Hake                  |         |
| 3,894,958 A     |   | 7/1975  | McCoy et al.          |         |
| 3,933,663 A     | * | 1/1976  | Thompson et al. ....  | 508/555 |
| 3,953,346 A     | * | 4/1976  | Thompson              | 508/555 |
| 4,002,569 A     | * | 1/1977  | Rubin et al.          | 508/476 |
| 4,141,848 A     | * | 2/1979  | Braid                 | 508/477 |
| 4,371,446 A     | * | 2/1983  | Kinoshita et al. .... | 508/144 |
| 4,581,039 A     |   | 4/1986  | Horodysky             |         |
| 4,789,493 A     |   | 12/1988 | Horodosky             |         |
| 5,344,579 A     |   | 9/1994  | Ohtani et al.         |         |
| 5,395,539 A     |   | 3/1995  | Chandler et al.       |         |
| 5,441,656 A     |   | 8/1995  | Ohtani et al.         |         |
| 5,628,804 A     |   | 5/1997  | Loper                 |         |
| 5,916,852 A     |   | 6/1999  | Nibert et al.         |         |
| 7,973,000 B2    | * | 7/2011  | Shitara et al. ....   | 508/551 |
| 2005/0082139 A1 |   | 4/2005  | Ishikawa et al.       |         |
| 2006/0058202 A1 |   | 3/2006  | Levine et al.         |         |
| 2008/0146468 A1 |   | 6/2008  | Konishi et al.        |         |
| 2009/0005277 A1 |   | 1/2009  | Watts et al.          |         |
| 2010/0210490 A1 |   | 8/2010  | Vickerman et al.      |         |

**FOREIGN PATENT DOCUMENTS**

|    |            |        |
|----|------------|--------|
| DE | 2529167    | 1/1977 |
| GB | 1505266    | 3/1978 |
| WO | 2010096325 | 8/2010 |

**OTHER PUBLICATIONS**

Corresponding PCT Publication and Search Report No. WO 2010/096321 published Aug. 26, 2010.

Written Opinion from corresponding PCT Application No. PCT/US2010/023855 mailed Jun. 22, 2010.

\* cited by examiner

*Primary Examiner* — Ellen McAvoy

(74) *Attorney, Agent, or Firm* — David M. Shold, Esq.; Michael F. Esposito, Esq.

(57) **ABSTRACT**

A composition is provided suitable for use as a friction modifier for an automatic transmission, comprising an N-substituted oxalic acid bisamide or amide-ester containing at least two hydrocarbyl groups of 12 to 22 carbon atoms.

**12 Claims, No Drawings**

**OXALIC ACID BIS-AMIDES OR  
AMIDE-ESTER AS FRICTION MODIFIERS IN  
LUBRICANTS**

**BACKGROUND OF THE INVENTION**

The present invention relates to the field of additives for fluids such as automatic transmission fluids, manual transmission fluids, traction fluids, fluids for continuously variable transmission fluids (CVTs), dual clutch automatic transmission fluids, farm tractor fluids, gear oils, and engine lubricants.

In the automatic transmission marketplace, where there is rapid engineering change driven by the desire to reduce weight and increase transmission capacity, there is a desire for automatic transmission fluids that exhibit a high static coefficient of friction for improved clutch holding capacity. Continuously slipping torque converter clutches, for instance, impose exacting friction requirements on automatic transmission fluids (ATFs). The fluid must have a good friction versus sliding speed relationship, or an objectionable phenomenon called shudder will occur in the vehicle. Transmission shudder is a self-excited vibrational state commonly called "stick-slip" or "dynamic frictional vibration" generally occurring in slipping torque converter clutches. The friction characteristics of the fluid and material system, combined with the mechanical design and controls of the transmission, determine the susceptibility of the transmission to shudder. Plotting the measured coefficient of friction ( $\mu$ ) versus sliding speed (V), commonly called a  $\mu$ -V curve, has been shown to correlate to transmission shudder. Both theory and experiments support the region of positive to slightly negative slope of this  $\mu$ -V curve to correlate to good anti-shudder performance of transmission fluids. A fluid which allows the vehicle to operate without vibration or shudder is said to have good "anti-shudder" performance. The fluid should maintain those characteristics over its service lifetime. The longevity of the anti-shudder performance in the vehicle is commonly referred to as "anti-shudder durability". The variable speed friction tester (VSFT) measures the coefficient of friction with respect to sliding speed simulating the speeds, loads, and friction materials found in transmission clutches and correlates to the performance found in actual use. The procedures are well documented in the literature; see for example Society of Automotive Engineers publication #941883.

The combined requirements of high static coefficient of friction and durable positive slope are often incompatible with traditional ATF friction modifier technology which is extremely well described in the patent literature. Many of the commonly used friction modifiers result in a low static coefficient of friction and are not durable enough on positive slope to be of sufficient use.

U.S. Pat. No. 5,395,539, Chandler et al., Mar. 7, 1995, discloses an amide containing friction modifier for use in power transmission fluids. The additive comprises a Component-1 formed by condensing a polyamine with an aliphatic monoacid.

U.S. Patent Application 2006/0058202, Levine et al., published Mar. 16, 2006, discloses certain amine derivatives of N-alkyl-halo-acetamides, which may be of the formula



where R, each independently, is alkyl or alkenyl of 1 to 8 carbon atoms.

U.S. Pat. No. 4,789,493, Horodysky, Dec. 6, 1988, discloses lubricants containing N-alkylalkylenediamine amides.

5 Disclosed is  $R^2-N(R^3)-R^1-NH-R^3$  wherein  $R^1$  is a  $C_2$  to  $C_4$  alkylene group,  $R^2$  must be a  $C_{12}$  to  $C_{30}$  hydrocarbyl group, and  $R^3$  is H, a  $C_1$ - $C_3$  aliphatic group, or  $R^4-C(=O)-$ ; at least one of the  $R^3$ 's must be  $R^4-C(=O)-$ .  $R^4$  is H or  $C_{1-4}$ . An example is Coco-NH-(CH<sub>2</sub>)<sub>3</sub>-NH-C(=O)H.

10 U.S. Pat. No. 4,581,039, Horodysky, Apr. 8, 1986 discloses lubricants containing N-hydrocarbyl hydrocarbylenediamine carboxylates, for example, the reaction product of N-oleyl-1, 3-propylenediamine with oleic acid. These are reported to have the formula



20 U.S. Pat. No. 5,344,579, Ohtani et al., Sep. 6, 1994, discloses a friction modifier system comprising a hydroxylalkyl aliphatic imidazoline, having on the 1-position on the ring a hydroxylalkyl group that contains from 2 to about 4 carbon atoms, and having in the adjacent 2-position on the ring a non-cyclic hydrocarbyl group containing about 10 to about 25 carbon atoms. A suitable compound is 1-hydroxyethyl-2-heptadecenyl imidazoline. Another component is a di(hydroxylalkyl)aliphatic tertiary amine. The hydrocarbyl group contains about 10 to about 25 carbon atoms. The hydroxylalkyl groups may be 2-hydroxyethyl groups.

25 35 U.S. Pat. No. 5,441,656, Ohtani et al., Aug. 15, 1995, discloses a friction modifier system that consists essentially of (i) an N-aliphatic hydrocarbyl-substituted diethanolamine and (ii) an N-aliphatic hydrocarbyl substituted trimethylene-diamine.

30 40 U.S. Pat. No. 3,251,853, Hoke, May 17, 1966, discloses an oil-soluble acylated amine. In examples, reactants can xylol-stearic acid or heptylphenylheptanoic acid, with tetraethylene pentamine or dodecylamine or N-2-aminoethyleoctadecylamine. An example is the condensation product of N-2-aminoethyl)octadecylamine with xylol-stearic acid.

45 50 55 U.S. Pat. No. 5,916,852, Nibert et al., Jun. 29, 1999, discloses a power transmission fluid composition comprising, among others, an amine (i.e., alkyl primary amine) having the structure R-NH<sub>2</sub> where R is about a C<sub>8</sub> to C<sub>30</sub> alkyl. It may also include an amine containing friction modifier. The amine may be, among others, tallow amine. The amine containing friction modifier may be the reaction products of a long chain carboxylic acid (such as, e.g., stearic acid) with a polyamine, and may be of the structure



55 60 or may be an alkoxylated amine such as those produced by reacting a long chain primary amine with a low molecular weight alkoxide such as ethylene oxide or propylene oxide.

65 U.S. Patent publication 2009/0005277, Watts et al., Jan. 1, 2009, discloses lubricating oil compositions said to have excellent friction stability, comprising, among other components, a polyalkylene polyamine-based friction modifier that

has been reacted with an acylating agent to convert at least one secondary amine group into an amide.

The disclosed technology, therefore, provides a friction modifier suitable for providing an automatic transmission fluid with a high coefficient of friction or a durable positive slope in a  $\mu$ -V curve or both.

#### SUMMARY OF THE INVENTION

The disclosed technology provides a composition, suitable for use as a friction modifier for a transmission, comprising an oil of lubricating viscosity and an N-substituted oxalic acid bisamide or amide-ester containing at least two hydrocarbyl groups of 12 to 22 carbon atoms. In certain embodiments, the bisamide or amide-ester does not contain a primary amino group.

The composition, which may be a lubricant, further comprises an oil of lubricating viscosity and may comprise one or more further additives, may be used in a method for lubricating a transmission such as an automatic transmission, comprising supplying the lubricant thereto.

#### DETAILED DESCRIPTION OF THE INVENTION

Various features and embodiments will be described below by way of non-limiting illustration.

One component which is used in certain embodiments of the disclosed technology is an oil of lubricating viscosity, which can be present in a major amount, for a lubricant composition, or in a concentrate forming amount, for a concentrate. Suitable oils include natural and synthetic lubricating oils and mixtures thereof. In a fully formulated lubricant, the oil of lubricating viscosity is generally present in a major amount (i.e. an amount greater than 50 percent by weight). Typically, the oil of lubricating viscosity is present in an amount of 75 to 95 percent by weight, and often greater than 80 percent by weight of the composition.

Natural oils useful in making the inventive lubricants and functional fluids include animal oils and vegetable oils as well as mineral lubricating oils such as liquid petroleum oils and solvent-treated or acid-treated mineral lubricating oils of the paraffinic, naphthenic or mixed paraffinic-/naphthenic types which may be further refined by hydrocracking and hydrofinishing processes.

Synthetic lubricating oils include hydrocarbon oils and halo-substituted hydrocarbon oils such as polymerized and interpolymerized olefins, also known as polyalphaolefins; polyphenyls; alkylated diphenyl ethers; alkyl- or dialkylbenzenes; and alkylated diphenyl sulfides; and the derivatives, analogs and homologues thereof. Also included are alkylene oxide polymers and inter-polymers and derivatives thereof, in which the terminal hydroxyl groups may have been modified by esterification or etherification. Also included are esters of dicarboxylic acids with a variety of alcohols, or esters made from C5 to C12 monocarboxylic acids and polyols or polyol ethers. Other synthetic oils include silicon-based oils, liquid esters of phosphorus-containing acids, and polymeric tetrahydrofurans.

Unrefined, refined and rerefined oils, either natural or synthetic, can be used in the lubricants of the present invention. Unrefined oils are those obtained directly from a natural or synthetic source without further purification treatment. Refined oils have been further treated in one or more purification steps to improve one or more properties. They can, for example, be hydrogenated, resulting in oils of improved stability against oxidation.

In one embodiment, the oil of lubricating viscosity is an API Group I, Group II, Group III, Group IV, or Group V oil, including a synthetic oil, or mixtures thereof. In another embodiment, the oil is Groups II, III, IV, or V. These are 5 classifications established by the API Base Oil Interchangeability Guidelines. Group III oils contain <0.03 percent sulfur and >90 percent saturates and have a viscosity index of >120. Group II oils have a viscosity index of 80 to 120 and contain <0.03 percent sulfur and >90 percent saturates. Polyalphaolefins are categorized as Group IV. The oil can also be an oil derived from hydroisomerization of wax such as slack wax or a Fischer-Tropsch synthesized wax. Such "Gas-to-Liquid" oils are typically characterized as Group III. Group V is 10 encompasses "all others" (except for Group I, which contains >0.03% S and/or <90% saturates and has a viscosity index of 80 to 120).

In one embodiment, at least 50% by weight of the oil of lubricating viscosity is a polyalphaolefin (PAO). Typically, 15 the polyalphaolefins are derived from monomers having from 4 to 30, or from 4 to 20, or from 6 to 16 carbon atoms. Examples of useful PAOs include those derived from 20 1-decene. These PAOs may have a viscosity of 1.5 to 150 mm<sup>2</sup>/s (cSt) at 100° C. PAOs are typically hydrogenated materials.

The oils of the present technology can encompass oils of a single viscosity range or a mixture of high viscosity and low viscosity range oils. In one embodiment, the oil exhibits a 25 100° C. kinematic viscosity of 1 or 2 to 8 or 10 mm<sup>2</sup>/sec (cSt). The overall lubricant composition may be formulated using 30 oil and other components such that the viscosity at 100° C. is 1 or 1.5 to 10 or 15 or 20 mm<sup>2</sup>/sec and the Brookfield viscosity (ASTM-D-2983) at -40° C. is less than 20 or 15 Pa-s (20,000 cP or 15,000 cP), such as less than 10 Pa-s, even 5 or less.

The present technology provides, as one component, an 35 N-substituted oxalic acid bisamide or amide-ester containing at least two hydrocarbyl groups of 12 to 22 carbon atoms. In certain embodiments, the compound does not contain a primary amine group. (This may be absent in any of the embodiments whatever the detailed chemical nature, and in the presence or absence of other components.) This material is useful 40 as a friction modifier, particularly for lubricating automatic transmissions. This component, as the bisamide, may be represented by the formula

45



In this structure at least two of the Rs are independently 50 groups comprising a hydrocarbyl group of 1 to 22 carbon atoms and up to two of the R groups are hydrogen or a hydrocarbyl group of 10 or fewer carbon atoms. In other embodiments, one or more of the R groups may independently contain 12 to 20 or 12 to 18 or 12 to 16 or 12 to 14 or 14 to 20 or 14 to 18 or 14 to 16 carbon atoms. If there are two 55 hydrocarbyl groups of 12 to 22 carbon atoms, they may be both on the same nitrogen or they may be on different nitrogen atoms; that is, either R<sup>3</sup> and R<sup>4</sup> or alternatively R<sup>3</sup> and R<sup>4</sup> may be hydrogen. The hydrocarbyl groups may be the same or different within a given molecule or within a mixture of molecules in the overall composition.

Since at least two of the groups R<sup>1</sup>, R<sup>2</sup>, R<sup>3</sup> and R<sup>4</sup> comprise 60 a hydrocarbyl group of 12 to 22 carbon atoms, such groups

may be such a hydrocarbyl group, for instance, an alkyl group of 12 to 22 carbon atoms. Alternatively, such groups may comprise such a hydrocarbyl group as a part of a larger structure. That is, such groups may have the general structure such as  $R^5R^6N-R^9$ —where one or both of the  $R^5$  and  $R^6$  are hydrocarbyl groups of 12 to 22 carbons and optionally one of the  $R^5$  and  $R^6$  may be hydrogen or a shorter hydrocarbyl group.  $R^9$  would be a hydrocarbylene linking group, such as methylene, ethylene, propylene, or butylene, and in some cases a 1-3-propylene group.

In some embodiments, therefore, the substituted oxalic acid bisamide may comprise a material of the structure about in which two of the groups  $R^1$ ,  $R^2$ ,  $R^4$ , and  $R^8$  are independently alkyl groups of about 12 to about 22 carbon atoms. Such materials may have a structure such as



wherein each  $R^1$  and  $R^2$  is independently an alkyl group of about 12 to about 18 carbon atoms. Such a material may be obtained or obtainable by known methods such as the process of reacting a dialkylamine with an alkyl oxamate such as ethyl oxamate.

In another embodiment, the N-substituted oxalic acid bisamide or amide-ester comprises an amide-ester represented by the formula:



In this embodiment,  $R^1$  and  $R^2$  may independently be hydrocarbyl groups of 12 to 22 carbon atoms, as defined elsewhere herein, and  $R^{10}$  may be a hydrocarbyl group of 1 to 22 carbon atoms. In certain embodiments,  $R^{10}$  is methyl, ethyl, n-propyl, isopropyl, n-butyl, sec-butyl, isobutyl, or t-butyl.

Long chain monoalkyl and dialkyl amines are commercially available. The hydrocarbyl group or groups of the amines may be described as long chain hydrocarbyl groups, by which is meant generally hydrocarbyl groups containing 12 to 22 carbon atoms. For monoalkyl amines, that is, primary amines, the hydrocarbyl group may comprise a mixture of individual groups on different molecules having a variety of carbon numbers falling generally within the range of 12 to 22 carbon atoms, although molecules with hydrocarbyl groups falling outside this range may also be present. If a mixture of hydrocarbyl groups is present, they may be primarily of even carbon number (e.g., 12, 14, 16, 18, 20, or 22) as is characteristic of groups derived from many naturally-occurring materials, or they may be a mixture of even and odd carbon numbers or, alternatively, an odd carbon number or a mixture of odd numbers. They may be branched, linear, or cyclic and may be saturated or unsaturated, or combinations thereof. In certain embodiments the hydrocarbyl groups may contain 16 to 18 carbon atoms, and sometimes predominantly 16 or predominantly 18. Specific examples include mixed "coco" groups, that is, cocoalkyl groups, from cocoamine (predominantly C12 and C14 amines) and mixed "tallow" groups, that

is, tallowalkyl groups, from tallowamine (predominantly C16 and C18 groups), and isostearyl groups. The tallow groups may optionally be hydrogenated. Likewise, dialkyl amines, that is, secondary amine, are commercially available, which may have one long chain alkyl group as described above and one short chain alkyl group of 1 to 10 carbon atoms, or which may have two long chain alkyl groups. Examples of the latter include dicocoamine (available as Armeen 2C<sup>TM</sup>), and ditallowamine. Others, such as isostearyl-coco amine may be synthesized generally as described for preparative example B below.

It is also contemplated that two or more of the groups  $R^1$ ,  $R^2$ ,  $R^3$ , and  $R^4$  may be independently N-hydrocarbyl-substituted or di-substituted aminoalkyl groups wherein the hydrocarbyl substituent or substituents contain 12 to 22 carbon atoms and the alkyl moieties contain 1 to 4 carbon atoms. A formula representing this general structure may be represented by

20



wherein  $R^5$  and  $R^7$  are independently a hydrocarbyl group of about 12 to about 22 carbon atoms and  $R^6$  and  $R^8$  are independently hydrogen or a hydrocarbyl group of 10 or fewer carbon atoms or a hydrocarbyl group of about 12 to about 22 carbon atoms. Diamines suitable for preparing such products include those in the "Duomeen" series, available from Akzo, having a general structure such as

35



Such polyamines may be prepared by the addition of the monoamine  $R^3R^4NH$  to acrylonitrile, to prepare the alkyl nitrile amine,

45



followed by catalytic reduction of the nitrile group using, e.g.,  $H_2$  over Pd/C catalyst, to give the diamine.

In a related embodiment, the N-substituted oxalic acid bisamide or amide-ester may comprise an amide-ester represented by the formula:

55



wherein  $R^5$  and  $R^6$  are independently hydrocarbyl groups of 12 to 22 carbon atoms as defined above and  $R^{10}$  may be a hydrocarbyl group of 1 to 22 carbon atoms, such as methyl, ethyl, n-propyl, isopropyl, n-butyl, sec-butyl, isobutyl, or t-butyl.

Some specific examples of the materials of the disclosed technology include those represented by the following structures:



where coco and tallow are as defined above and isostearyl represents the carbon architecture of isostearic acid.

The bisamides disclosed herein may be prepared by known techniques such as reaction of the appropriate amine with oxalic acid or a reactive equivalent thereof, such as ethyl oxamide or dimethyl oxalate, as illustrated in the preparative examples below. The amide-esters may be prepared by reaction of the appropriate amine with a dialkyl oxalate, using a controlled amount of amine (approximating 1:1 molar ratio) or by reacting the amine with the half ester-half chloride (e.g., ethyl 2-chloro-2-oxo-acetate). Minor amounts of the amide-esters may be formed along with the preparation of the bisamides, and the relative amounts may be adjusted by known techniques.

The amount of the amine in a fully formulated lubricant may be 0.1 to 10 percent by weight, or 0.5 to 6 percent or 0.8 to 4 percent, or 1 to 2.5 percent.

Other components may be present. One such component is a dispersant. It may be described as "other than an amine compound as described above" in the event that some of the amine compounds described above may exhibit some dispersant characteristics. Examples of "carboxylic dispersants" are described in many U.S. Patents including the following: U.S. Pat. Nos. 3,219,666, 3,316,177, 3,340,281, 3,351,552, 3,381,022, 3,433,744, 3,444,170, 3,467,668, 3,501,405, 3,542,680, 3,576,743, 3,632,511, 4,234,435, Re 26,433, and 6,165,235.

Succinimide dispersants, a species of carboxylic dispersants, are prepared by the reaction of a hydrocarbyl-substituted succinic anhydride (or reactive equivalent thereof, such as an acid, acid halide, or ester) with an amine, as described above.

5 The hydrocarbyl substituent group generally contains an average of at least 8, or 20, or 30, or 35 up to 350, or to 200, or to 100 carbon atoms. In one embodiment, the hydrocarbyl group is derived from a polyalkene. Such a polyalkene can be characterized by an  $M_n$  (number average molecular weight) 10 of at least 500. Generally, the polyalkene is characterized by an  $M_n$  of 500 or 700 or 800 or 900, up to 5000 or to 2500 or to 2000 or to 1500. In another embodiment  $M_n$  varies from 500 or 700 or 800, to 1200 or 1300. In one embodiment the polydispersity ( $M_w/M_n$ ) is at least 1.5.

15 The polyalkenes include homopolymers and inter-polymers of polymerizable olefin monomers of 2 to 16 or to 6, or to 4 carbon atoms. The olefins may be monoolefins such as ethylene, propylene, 1-butene, isobutene, and 1-octene; or a polyolefinic monomer, such as diolefinic monomer, such 20 1,3-butadiene and isoprene. In one embodiment, the polymer is a homo-polymer. An example of a polymer is a polybutene. In one instance about 50% of the polybutene is derived from isobutylene. The polyalkenes can be prepared by conventional procedures.

25 In one embodiment, the succinic acylating agents are prepared by reacting a polyalkene with an excess of maleic anhydride to provide substituted succinic acylating agents wherein the number of succinic groups for each equivalent weight of substituent group is at least 1.3, e.g., 1.5, or 1.7, or

30 1.8. The maximum number of succinic groups per substituent group generally will not exceed 4.5, or 2.5, or 2.1, or 2.0. The preparation and use of substituted succinic acylating agents wherein the substituent is derived from such polyolefins are described in U.S. Pat. No. 4,234,435.

35 The substituted succinic acylating agent can be reacted with an amine, including those amines described above and heavy amine products known as amine still bottoms. The amount of amine reacted with the acylating agent is typically an amount to provide a mole ratio of CO:N of 1:2 to 1:0.25, or 40 1:2 to 1:0.75. If the amine is a primary amine, complete condensation to the imide can occur. Varying amounts of amide product, such as the amide acid, may also be present. If the reaction is, rather, with an alcohol, the resulting dispersant will be an ester dispersant. If both amine and alcohol 45 functionality are present, whether in separate molecules or in the same molecule (as in the above-described condensed amines), mixtures of amide, ester, and possibly imide functionality can be present. These are the so-called ester-amide dispersants.

50 "Amine dispersants" are reaction products of relatively high molecular weight aliphatic or alicyclic halides and amines, such as polyalkylene polyamines. Examples thereof are described in the following U.S. Pat. Nos. 3,275,554, 3,438,757, 3,454,555, and 3,565,804.

55 "Mannich dispersants" are the reaction products of alkyl phenols in which the alkyl group contains at least 30 carbon atoms with aldehydes (especially formaldehyde) and amines (especially polyalkylene polyamines). The materials described in the following U.S. Patents are illustrative: U.S. 60 Pat. Nos. 3,036,003, 3,236,770, 3,414,347, 3,448,047, 3,461, 172, 3,539,633, 3,586,629, 3,591,598, 3,634,515, 3,725,480, 3,726,882, and 3,980,569.

Post-treated dispersants are also part of the present invention. They are generally obtained by reacting carboxylic, 65 amine or Mannich dispersants with reagents such as urea, thiourea, carbon disulfide, aldehydes, ketones, carboxylic acids, hydrocarbon-substituted succinic anhydrides, nitriles,

epoxides, boron compounds such as boric acid (to give "borated dispersants"), phosphorus compounds such as phosphorus acids or anhydrides, or 2,5-dimercaptothiadiazole (DMTD). Exemplary materials of this kind are described in the following U.S. Pat. Nos. 3,200,107, 3,282,955, 3,367, 943, 3,513,093, 3,639,242, 3,649,659, 3,442,808, 3,455,832, 3,579,450, 3,600,372, 3,702,757, and 3,708,422.

Mixtures of dispersants can also be used. The amount of dispersant or dispersants, if present in formulations of the present technology, is generally 0.3 to 10 percent by weight. In other embodiments, the amount of dispersant is 0.5 to 7 percent or 1 to 5 percent of the final blended fluid formulation. In a concentrate, the amounts will be proportionately higher.

Another component frequently used is a viscosity modifier. Viscosity modifiers (VM) and dispersant viscosity modifiers (DVM) are well known. Examples of VMs and DVMs may include polymethacrylates, polyacrylates, polyolefins, styrene-maleic ester copolymers, and similar polymeric substances including homopolymers, copolymers and graft copolymers. The DVM may comprise a nitrogen-containing methacrylate polymer, for example, a nitrogen-containing methacrylate polymer derived from methyl methacrylate and dimethylaminopropyl amine.

Examples of commercially available VMs, DVMs and their chemical types may include the following: polyisobutylenes (such as Indopol<sup>TM</sup> from BP Amoco or Parapol<sup>TM</sup> from ExxonMobil); olefin copolymers (such as Lubrizol<sup>TM</sup> 7060, 7065, and 7067 from Lubrizol and Lucant<sup>TM</sup> HC-2000L and HC-600 from Mitsui); hydrogenated styrene-diene copolymers (such as Shellvis<sup>TM</sup> 40 and 50, from Shell and LZ<sup>®</sup> 7308, and 7318 from Lubrizol); styrene/maleate copolymers, which are dispersant copolymers (such as LZ<sup>®</sup> 3702 and 3715 from Lubrizol); polymethacrylates, some of which have dispersant properties (such as those in the Viscoplex<sup>TM</sup> series from RohMax, the Hitec<sup>TM</sup> series from Afton, and LZ 7702<sup>TM</sup>, LZ 7727<sup>TM</sup>, LZ 7725<sup>TM</sup> and LZ 7720C<sup>TM</sup> from Lubrizol); olefin-graft-polymethacrylate polymers (such as Viscoplex<sup>TM</sup> 2-500 and 2-600 from RohMax); and hydrogenated polyisoprene star polymers (such as Shellvis<sup>TM</sup> 200 and 260, from Shell). Also included are Asteric<sup>TM</sup> polymers from Lubrizol (methacrylate polymers with radial or star architecture). Viscosity modifiers that may be used are described in U.S. Pat. Nos. 5,157,088, 5,256,752 and 5,395,539. The VMs and/or DVMs may be used in the functional fluid at a concentration of up to 20% by weight. Concentrations of 1 to 12%, or 3 to 10% by weight may be used.

Another component that may be used in the composition used in the present technology is a supplemental friction modifier. These friction modifiers are well known to those skilled in the art. A list of friction modifiers that may be used is included in U.S. Pat. Nos. 4,792,410, 5,395,539, 5,484,543 and 6,660,695. U.S. Pat. No. 5,110,488 discloses metal salts of fatty acids and especially zinc salts, useful as friction modifiers. A list of supplemental friction modifiers that may be used may include:

-continued

|                                      |                             |
|--------------------------------------|-----------------------------|
| hydroxyalkyl amides                  | polyhydroxy tertiary amines |
| and mixtures of two or more thereof. |                             |

5 Representatives of each of these types of friction modifiers are known and are commercially available. For instance, fatty phosphites may be generally of the formula  $(RO)_2PHO$  or  $(RO)(HO)PHO$  where R may be an alkyl or alkenyl group of sufficient length to impart oil solubility. Suitable phosphites are available commercially and may be synthesized as described in U.S. Pat. No. 4,752,416.

10 Borated fatty epoxides that may be used are disclosed in Canadian Patent No. 1,188,704. These oil-soluble boron-containing compositions may be prepared by reacting a boron source such as boric acid or boron trioxide with a fatty epoxide which may contain at least 8 carbon atoms. Non-borated fatty epoxides may also be useful as supplemental friction modifiers.

15 20 Borated amines that may be used are disclosed in U.S. Pat. No. 4,622,158. Borated amine friction modifiers (including borated alkoxylated fatty amines) may be prepared by the reaction of a boron compounds, as described above, with the corresponding amines, including simple fatty amines and hydroxy containing tertiary amines. The amines useful for preparing the borated amines may include commercial alkoxylated fatty amines known by the trademark "ETHOMEEN" and available from Akzo Nobel, such as bis[2-hydroxyethyl]-cocoamine, polyoxyethylene[10]cocoamine, bis[2-hydroxyethyl]-soyamine, bis[2-hydroxyethyl]allowamine, polyoxyethylene-[5]tallowamine, bis[2-hydroxyethyl]oleylamine, bis[2-hydroxyethyl]octadecylamine, and polyoxyethylene[15]octadecylamine. Such amines are described in U.S. Pat. No. 4,741,848.

25 30 Alkoxylated fatty amines and fatty amines themselves (such as oleylamine) may be useful as friction modifiers. These amines are commercially available.

35 Both borated and unborated fatty acid esters of glycerol may be used as friction modifiers. Borated fatty acid esters of glycerol may be prepared by borating a fatty acid ester of glycerol with a boron source such as boric acid. Fatty acid esters of glycerol themselves may be prepared by a variety of methods well known in the art. Many of these esters, such as glycerol monooleate and glycerol tallowate, are manufactured on a commercial scale. Commercial glycerol monooleates may contain a mixture of 45% to 55% by weight mono-ester and 55% to 45% by weight diester.

40 45 Fatty acids may be used in preparing the above glycerol esters; they may also be used in preparing their metal salts, amides, and imidazolines, any of which may also be used as friction modifiers. The fatty acids may contain 6 to 24 carbon atoms, or 8 to 18 carbon atoms. A useful acid may be oleic acid.

50 55 The amides of fatty acids may be those prepared by condensation with ammonia or with primary or secondary amines such as diethylamine and diethanolamine. Fatty imidazolines may include the cyclic condensation product of an acid with a diamine or polyamine such as a polyethylenepolyamine. In one embodiment, the friction modifier may be the condensation product of a C8 to C24 fatty acid with a polyalkylene polyamine, for example, the product of isostearic acid with tetraethylenepentamine. The condensation products of carboxylic acids and polyalkyleneamines may be imidazolines or amides.

60 65 65 The fatty acid may also be present as its metal salt, e.g., a zinc salt. These zinc salts may be acidic, neutral or basic (overbased). These salts may be prepared from the reaction of

|                                                          |                                                                       |
|----------------------------------------------------------|-----------------------------------------------------------------------|
| fatty phosphites                                         | borated alkoxylated fatty amines                                      |
| fatty acid amides                                        | metal salts of fatty acids                                            |
| fatty epoxides                                           | sulfurized olefins                                                    |
| borated fatty epoxides                                   | fatty imidazolines                                                    |
| fatty amines other than the fatty amines discussed above | condensation products of carboxylic acids and polyalkylene-polyamines |
| glycerol esters                                          | metal salts of alkyl salicylates                                      |
| borated glycerol esters                                  | amine salts of alkylphosphoric acids                                  |
| alkoxylated fatty amines                                 | ethoxylated alcohols                                                  |
| oxazolines                                               | imidazolines                                                          |

a zinc containing reagent with a carboxylic acid or salt thereof. A useful method of preparation of these salts is to react zinc oxide with a carboxylic acid. Useful carboxylic acids are those described herein-above. Suitable carboxylic acids include those of the formula RCOOH where R is an aliphatic or alicyclic hydrocarbon radical. Among these are those wherein R is a fatty group, e.g., stearyl, oleyl, linoleyl, or palmityl. Also suitable are the zinc salts wherein zinc is present in a stoichiometric excess over the amount needed to prepare a neutral salt. Salts wherein the zinc is present from 1.1 to 1.8 times the stoichiometric amount, e.g., 1.3 to 1.6 times the stoichiometric amount of zinc, may be used. These zinc carboxylates are known in the art and are described in U.S. Pat. No. 3,367,869. Metal salts may also include calcium salts. Examples may include overbased calcium salts.

Sulfurized olefins are also well known commercial materials used as friction modifiers. A suitable sulfurized olefin is one which is prepared in accordance with the detailed teachings of U.S. Pat. Nos. 4,957,651 and 4,959,168. Described therein is a cosulfurized mixture of 2 or more reactants selected from the group consisting of at least one fatty acid ester of a polyhydric alcohol, at least one fatty acid, at least one olefin, and at least one fatty acid ester of a monohydric alcohol. The olefin component may be an aliphatic olefin, which usually will contain 4 to 40 carbon atoms. Mixtures of these olefins are commercially available. The sulfurizing agents useful in the process of the present invention include elemental sulfur, hydrogen sulfide, sulfur halide plus sodium sulfide, and a mixture of hydrogen sulfide and sulfur or sulfur dioxide.

Metal salts of alkyl salicylates include calcium and other salts of long chain (e.g. C12 to C16) alkyl-substituted salicylic acids.

Amine salts of alkylphosphoric acids include salts of oleyl and other long chain esters of phosphoric acid, with amines such as tertiary-aliphatic primary amines, sold under the trademark Primene™.

The amount of the supplemental friction modifier, if it is present, may be 0.1 to 1.5 percent by weight of the lubricating composition, such as 0.2 to 1.0 or 0.25 to 0.75 percent. In some embodiments, however, the amount of the supplemental friction modifier is present at less than 0.2 percent or less than 0.1 percent by weight, for example, 0.01 to 0.1 percent.

The compositions of the present technology can also include a detergent. Detergents as used herein are metal salts of organic acids. The organic acid portion of the detergent is a sulfonate, carboxylate, phenate, salicylate. The metal portion of the detergent is an alkali or alkaline earth metal. Suitable metals include sodium, calcium, potassium and magnesium. Typically, the detergents are overbased, meaning that there is a stoichiometric excess of metal base over that needed to form the neutral metal salt.

Suitable overbased organic salts include the sulfonate salts having a substantially oleophilic character and which are formed from organic materials. Organic sulfonates are well known materials in the lubricant and detergent arts. The sulfonate compound should contain on average 10 to 40 carbon atoms, such as 12 to 36 carbon atoms or 14 to 32 carbon atoms on average. Similarly, the phenates, salicylates, and carboxylates have a substantially oleophilic character.

While the present invention allows for the carbon atoms to be either aromatic or in paraffinic configuration, in certain embodiments alkylated aromatics are employed. While naphthalene based materials may be employed, the aromatic of choice is the benzene moiety.

Suitable compositions thus include an overbased monosulfonated alkylated benzene such as a monoalkylated benzene.

Typically, alkyl benzene fractions are obtained from still bottom sources and are mono- or di-alkylated. It is believed, in the present invention, that the mono-alkylated aromatics are superior to the dialkylated aromatics in overall properties.

It is sometimes desired that a mixture of mono-alkylated aromatics (benzene) be utilized to obtain the mono-alkylated salt (benzene sulfonate) in the present invention. The mixtures wherein a substantial portion of the composition contains polymers of propylene as the source of the alkyl groups may assist in the solubility of the salt. The use of mono-functional (e.g., monosulfonated) materials avoids crosslinking of the molecules with less precipitation of the salt from the lubricant. It is also frequently desired to use an alkylated benzene prepared by alkylation with an  $\alpha$ -olefin.

The salt may be "overbased." By overbasing, it is meant that a stoichiometric excess of the metal base be present over that required for the anion of the neutral salt. The excess metal from overbasing has the effect of neutralizing acids which may build up in the lubricant. Typically, the excess metal will be present over that which is required to neutralize the anion at in the ratio of up to 30:1, such as 5:1 to 18:1 on an equivalent basis.

The amount of the overbased salt utilized in the composition is typically 0.025 to 3 weight percent on an oil free basis, such as 0.1 to 1.0 percent. In other embodiments, the final lubricating composition may contain no detergent or substantially no detergent or only a low amount of detergent. That is, for a calcium overbased detergent for instance, the amount may be such as to provide less than 250 parts per million calcium, e.g., 0 to 250 or 1 to 200 or 10 to 150 or 20 to 100 or 30 to 50 parts per million calcium, or less than any of the foregoing non-zero amounts. This is in contrast with more conventional formulations which may contain sufficient calcium detergent to provide 300 to 600 ppm calcium. The overbased salt usually has up to about 50% oil and has a TBN range of 10-800 or 10-600 on an oil free basis. Borated and non-borated overbased detergents are described in U.S. Pat. Nos. 5,403,501 and 4,792,410.

The compositions of the present invention can also include at least one phosphorus acid, phosphorus acid salt, phosphorus acid ester or derivative thereof including sulfur-containing analogs in the amount of 0.002-1.0 weight percent. The phosphorus acids, salts, esters or derivatives thereof include phosphoric acid, phosphorous acid, phosphorus acid esters or salts thereof, phosphites, phosphorus-containing amides, phosphorus-containing carboxylic acids or esters, phosphorus-containing ethers, and mixtures thereof.

In one embodiment, the phosphorus acid, ester or derivative can be an organic or inorganic phosphorus acid, phosphorus acid ester, phosphorus acid salt, or derivative thereof. The phosphorus acids include the phosphoric, phosphonic, phosphinic, and thiophosphoric acids including dithiophosphoric acid as well as the mono thiophosphoric, thiophosphinic and thiophosphonic acids. One group of phosphorus compounds are alkylphosphoric acid mono alkyl primary amine salts as represented by the formula



where  $\text{R}^1, \text{R}^2, \text{R}^3$  are alkyl or hydrocarbyl groups or one of  $\text{R}^1$  and  $\text{R}^2$  can be H. The materials can be a 1:1 mixture of dialkyl

## 13

and monoalkyl phosphoric acid esters. Compounds of this type are described in U.S. Pat. No. 5,354,484.

Eighty-five percent phosphoric acid is a suitable material for addition to the fully-formulated compositions and can be included at a level of 0.01-0.3 weight percent based on the weight of the composition, such as 0.03 to 0.2 or to 0.1 percent.

Other phosphorus-containing materials that may be present include dialkylphosphites (sometimes referred to as dialkyl hydrogen phosphonates) such as dibutyl phosphite. Yet other phosphorus materials include phosphorylated hydroxy-substituted triesters of phosphorothioic acids and amine salts thereof, as well as sulfur-free hydroxy-substituted di-esters of phosphoric acid, sulphur-free phosphorylated hydroxy-substituted di- or tri-esters of phosphoric acid, and amine salts thereof. These materials are further described in U.S. patent application US 2008-0182770.

Other materials can optionally be included in the compositions of the present technology, provided that they are not incompatible with the aforementioned required components or specifications. Such materials include antioxidants (that is, oxidation inhibitors), including hindered phenolic antioxidants, secondary aromatic amine antioxidants such as dinonyldiphenylamine as well as such well-known variants as monononyldiphenylamine and diphenylamines with other alkyl substituents such as mono- or di-ocyl, sulfurized phenolic antioxidants, oil-soluble copper compounds, phosphorus-containing antioxidants, and organic sulfides, disulfides, and polysulfides such as 2-hydroxyalkyl, alkyl thioethers or 1-t-dodecylthio-2-propanol or sulfurized 4-carbobutoxy-cyclohexene or other sulfurized olefins. Also included may be corrosion inhibitors such as tolyl triazole and dimercaptothiadiazole and oil-soluble derivatives of such materials. Other optional components include seal swell compositions, such as isodecyl sulfolane or phthalate esters, which are designed to keep seals pliable. Also permissible are pour point depressants, such as alkynaphthalenes, polymethacrylates, vinyl acetate/fumarate or/maleate copolymers, and styrene/maleate copolymers. Other materials are an anti-wear agents such as zinc dialkyldithiophosphates, tridecyl adipate, and various long-chain derivatives of hydroxy carboxylic acids, such as tartrates, tartramides, tartrimides, and citrates as described in US Application 2006-0183647. These optional materials are known to those skilled in the art, are generally commercially available, and are described in greater detail in published European Patent Application 761,805. Also included can be known materials such as corrosion inhibitors (e.g., tolyltriazole, dimercaptothiadiazoles), dyes, fluidizing agents, odor masking agents, and antifoam agents. Organic borate esters and organic borate salts can also be included.

The above components can be in the form of a fully-formulated lubricant or in the form of a concentrate within a smaller amount of lubricating oil. If they are present in a concentrate, their concentrations will generally be directly proportional to their concentrations in the more dilute form in the final blend.

As used herein, the term "hydrocarbyl substituent" or "hydrocarbyl group" is used in its ordinary sense, which is well-known to those skilled in the art. Specifically, it refers to a group having a carbon atom directly attached to the remainder of the molecule and having predominantly hydrocarbon character. Examples of hydrocarbyl groups include:

hydrocarbon substituents, that is, aliphatic (e.g., alkyl or alkenyl), alicyclic (e.g., cycloalkyl, cycloalkenyl) substituents, and aromatic-, aliphatic-, and alicyclic-substituted aromatic substituents, as well as cyclic substituents wherein the

## 14

ring is completed through another portion of the molecule (e.g., two substituents together form a ring);

substituted hydrocarbon substituents, that is, substituents containing non-hydrocarbon groups which, in the context of this invention, do not alter the predominantly hydrocarbon nature of the substituent (e.g., halo (especially chloro and fluoro), hydroxy, alkoxy, mercapto, alkylmercapto, nitro, nitroso, and sulfoxyl);

10 hetero substituents, that is, substituents which, while having a predominantly hydrocarbon character, in the context of this invention, contain other than carbon in a ring or chain otherwise composed of carbon atoms and encompass substituents as pyridyl, furyl, thiienyl and imidazolyl. Heteroatoms include sulfur, oxygen, and nitrogen. In general, no more than two, or no more than one, heteroatom will be present for every ten carbon atoms in the hydrocarbyl group; typically, there will be no heteroatoms in the hydrocarbyl group.

15 It is known that some of the materials described above may interact in the final formulation, so that the components of the final formulation may be different from those that are initially added. For instance, metal ions (of, e.g., a detergent) can migrate to other acidic or anionic sites of other molecules. The products formed thereby, including the products formed upon employing the composition of the present invention in its intended use, may not be susceptible of easy description. Nevertheless, all such modifications and reaction products are included within the scope of the present invention; the present invention encompasses the composition prepared by admixing the components described above.

## EXAMPLES

More detailed preparative examples of several amino esters and subsequently amino amides are provided below. It is to be understood that in each instance the desired product may not be exactly represented by the formula indicated above. For instance, there may be greater or lesser amounts of mono- or di- or tri-substituted amines present in addition to the particular formula indicated. In some instances a product or byproduct other than that of the indicated structure may even be responsible for a significant portion of the activity of the product. Thus, the structures listed herein are not intended to be limiting.

## Preparative Example A

(To prepare the material represented by formula (I) above.) Dicocoamine (150 g) and xylene (550 mL) are combined with stirring under a nitrogen atmosphere. To this mixture, ethyl oxamate (58.6 g) is added in one portion. The mixture is heated to 110° C. and stirred for 7 hours, collecting ethanol in a Dean-Stark trap. The mixture is then heated to 135° C. and stirred for 5 hours, removing the xylene by distillation. The mixture is further heated to 155° C. and stirred for 7 hours, then allowed to cool and filtered through a glass fiber filter paper. Any remaining solvent is removed under reduced pressure using a rotary evaporator, leaving an orange oil product.

## Preparative Example B

(To prepare the material represented by formula (II) above.) Part 1, N-coco isostearamide. Isostearic acid (215 g) and xylene (1 L) are combined with stirring under a nitrogen atmosphere. Armeen C™ (156 g) is added in one portion and the mixture is stirred at 148° C. for 12 hours with removal of water (13.4 g) by azeotropic distillation using a Dean-Stark

## 15

trap. The mixture is allowed to cool and any remaining solvent is removed under reduced pressure using a rotary evaporator.

Part 2, isostearyl cocoamine. Lithium aluminum hydride (55 g) and dried tetrahydrofuran (THF, 1 L) are combined under nitrogen atmosphere and maintained at 0 to 10° C. The product from part 1, (330 g) is combined with 1 L dry THF and added to the reaction mixture over 40 minutes at 0 to 10° C. The mixture is stirred for 1 hour, then heated to reflux (67° C.) and stirred for 2 hours, then cooled to 0° C. Water (55 mL) is added dropwise over 3 hours, maintaining the temperature at 5 to 12° C. Methyl t-butyl ether (2 L) is then added with stirring, and the resulting mixture is dried over magnesium sulfate. The dried solution is filtered and concentrated under reduced pressure using a rotary evaporator.

Part 3. N-cocoyl-N-isostearyl-oxalamide. The product from part 2 (55.0 g) and xylene (350 mL) are combined with stirring under nitrogen. Ethyl oxamate (17.45 g) is added in one portion and the mixture is heated to 130° C., with stirring for 20 hours. The temperature is increased and solvent is removed by distillation. The mixture is further heated to 160° C. for 3 hours, then allowed to cool and filtered through glass fiber filter paper. Any remaining solvent is removed under reduced pressure using a rotary evaporator to provide the product.

## Preparative Example C

(To prepare the material represented by formula (III) above.) Duomeen C™ (112 g) and toluene (350 mL) are combined with stirring under a nitrogen atmosphere. Dimethyl oxalate (24.25 g) is added in one portion and the reaction is heated to 95° C. with stirring for 5 hours, removing methanol by azeotropic distillation using a Dean-Stark trap. The mixture is then heated to 105° C. with stirring for 4 hours. Any remaining solvent is removed under reduced pressure using a rotary evaporator.

Preparative example D (To prepare the material represented by formula (IV) above.) Duomeen 2HT™ (N,N-diallyl propylenediamine, 207.8 g) and toluene (400 mL) are combined with stirring under nitrogen. To this mixture, dimethyl oxalate (20.4 g) is added in one portion. The mixture is heated to 112° C. and stirred for 6½ hours. The mixture is further heated to 120° C. with stirring for 7 hours, then allowed to cool. Any remaining solvent is removed under reduced pressure using a rotary evaporation.

Alternatively, the above procedure is substantially repeated but using a 10% excess of dimethyl oxalate. Upon cooling, the reaction mixture solidifies and is then broken up and stirred in acetone for 4 hours. The slurry is filtered, the solid product is collected as the filter cake and the residual acetone is removed from the product under reduced pressure using a rotary evaporator.

Two base formulations are prepared in which certain of the above-described materials are tested.

## Base Formulation A:

3.5% succinimide dispersant(s) (containing 41.5% oil)  
0.2% dibutyl phosphite  
0.1% phosphoric acid  
0.1% borate ester  
0.9% amine antioxidant  
0.4% seal swell agent  
1.1% calcium sulfonate detergents (containing 50% oil)  
0.06% substituted thiadiazole  
0.2% pour point depressant  
0.04% ethoxylated amine  
9.6% dispersant viscosity modifier (containing 25% oil)

## 16

0.04% other minor components  
balance: mineral oils (predominantly 3-6 cSt)

## Base Formulation B:

3.5% succinimide dispersant(s) (containing 41.5% oil)  
5 0.2% dibutyl phosphite  
0.1% phosphoric acid  
0.9% amine antioxidant  
0.4% seal swell agent  
0.2% pour point depressant  
10 9.6% dispersant viscosity modifier (containing 25% oil)  
0.03% other minor components  
balance: mineral oils (predominantly 3-6 cSt)

Lubricants for testing are prepared by adding one of the materials from the preparative examples, identified in the tables below, to the indicated base formulation. The resulting lubricants are subjected to a VSFT test, which is a variable speed friction test. The VSFT apparatus consists of a disc that can be metal or another friction material which is rotated against a metal surface. The friction materials employed in the particular tests are various commercial friction materials commonly used in automatic transmission clutches, as indicated in the Tables. The test is run over three temperatures and two load levels. The coefficient of friction measured by the VSFT is plotted against the sliding speed (50 and 200 r.p.m.) over a number speed sweeps at a constant pressure. The results are initially presented as slope of the  $\mu$ -v curve as a function of time, reported for 40, 80, and 120° C. and 24 kg and 40 kg (235 and 392 N) force, determined at 4 hour intervals from 0 to 52 hours. Typically, the slope will initially be positive, with a certain amount of variability, and may gradually decrease, possibly becoming negative after a certain period of time. Longer duration of positive slope is desired.

The data is initially collected as a table of slope values as a function of time, for each run. For ease of analysis and comparison, each formulation at each temperature is assigned a "slope score." At each temperature, the fraction of slope values within the first 7 time measurements (0 to 24 hours) at 24 kg and of the first 7 measurements at 40 kg (thus 14 measurements total) that are positive, as a percent, is denoted as "A". The fraction of the slope values at the two pressures (14 measurements total) within the second 24 hours (28-52 hours) that are positive are denoted as "B". The slope score is defined as A+2B. The extra weighting given to the latter portion of the test is to reflect the greater importance (and difficulty) of preparing a durable fluid that retains a positive slope in the latter stages of the test. The maximum score of 300 denotes a fluid that exhibits a consistently positive slope through the entire test. For illustration, the individual slope results for Preparative Example A at 0.25% in Formulation A are presented below, along with the of the "slope score."

| Preparative Example A, 1%, 40° C., formulation A |          |                       |                       |                                  |
|--------------------------------------------------|----------|-----------------------|-----------------------|----------------------------------|
|                                                  | Time, hr | $\mu$ -V Slope, 24 kg | $\mu$ -V Slope, 40 kg | Slope Score (A + 2B)             |
| 60                                               | 0        | 0.007                 | 0.007                 | A = 14/14 = 100 + 2 × 64.3 = 229 |
|                                                  | 4        | 0.006                 | 0.006                 | 100%                             |
|                                                  | 8        | 0.007                 | 0.007                 |                                  |
|                                                  | 12       | 0.005                 | 0.006                 |                                  |
|                                                  | 16       | 0.006                 | 0.006                 |                                  |
|                                                  | 20       | 0.005                 | 0.006                 |                                  |
|                                                  | 24       | 0.002                 | 0.004                 |                                  |
| 65                                               | 28       | 0.002                 | 0.003                 | B = 9/14 = 64.3%                 |
|                                                  | 32       | 0.001                 | 0.004                 |                                  |
|                                                  | 36       | 0.001                 | 0.004                 |                                  |

## 17

-continued

| Preparative Example A, 1%, 40° C., formulation A |                  |                  |                      |
|--------------------------------------------------|------------------|------------------|----------------------|
| Time, hr                                         | μ-V Slope, 24 kg | μ-V Slope, 40 kg | Slope Score (A + 2B) |
| 40                                               | -0.002           | 0.003            |                      |
| 44                                               | -0.003           | 0.002            |                      |
| 48                                               | -0.004           | 0.001            |                      |
| 52                                               | -0.006           | 0.000            |                      |

A summary of the "slope scores" for certain of the materials of the present technology is provided in the table below:

| Ex.            | Ex.  | Prep | Treat, | Base | Friction | Slope Score        |                 |                  |
|----------------|------|------|--------|------|----------|--------------------|-----------------|------------------|
|                |      |      |        |      |          | Mat'l <sup>a</sup> | 40° C.          | 80° C.           |
| 1              | A    | 1    |        | A    | 4211     | 229                | 257             | 300              |
| 2              | A    | 2.5  |        | A    | 4211     | 293                | 257             | 264              |
| 3              | C    | 0.25 |        | A    | 7189     | 121                | 143             | 257              |
| 4              | C    | 1    |        | A    | 7189     | 107                | 157             | 200              |
| 5              | C    | 2.5  |        | A    | 7189     | 214                | 271             | 300              |
| X <sup>b</sup> | none | 0    |        | A    | 7189     | 19 <sup>c</sup>    | 95 <sup>c</sup> | 159 <sup>c</sup> |
| 6              | A    | 2.5  |        | B    | 4211     | 7                  | 100             | 171              |
| 7              | B    | 2.5  |        | B    | 6100     | 86                 | 164             | 164              |
| 8              | C    | 0.25 |        | B    | 7189     | 21                 | 57              | 157              |
| 9              | C    | 1    |        | B    | 7189     | 14                 | 50              | 229              |
| 10             | C    | 2.5  |        | B    | 7189     | 43                 | 86              | 129              |
| 11             | D    | 2.5  |        | B    | 4211     | 300                | 300             | 300              |
| 12             | D    | 2.5  |        | B    | 6100     | 300                | 300             | 300              |
| Y <sup>b</sup> | none | 0    |        | B    | 4211     | 0                  | 14              | 200              |
| Z <sup>b</sup> | none | 0    |        | B    | 7189     | 0                  | 0               | 64               |

<sup>a</sup>Friction materials: Raybestos™ 7911, Raybestos™ 4311, or Borg Warner™ 6100

<sup>b</sup>A reference example

<sup>c</sup>Average of 3 runs

The results show desirable frictional performance by materials of the present technology, in particular as compared to the base formulations from which they are absent. The results also indicate that better performance is sometimes obtained at relatively higher concentrations of 0.35 or 0.5 percent or greater, e.g., 1.0 or 2.5% compared with 0.25%. Even the relatively lower values for Example 6 are nevertheless better than those of Reference Example Y, particularly at 80° C.

Some of the materials tested exhibit exceptionally good performance. Especially noteworthy in this regard is the material of Preparative Example D, Formula (IV), which may be designated as N,N'-bis-(3-ditallowamino-propyl)-oxalamide. It is to be understood that some or all of the tallow groups in Formula (XII) and in the nomenclature may alternatively be coco groups or may be more generally represented by hydrocarbyl or alkyl groups of 12 to 22 carbon atoms.

Each of the documents referred to above is incorporated herein by reference. The mention of any document is not an admission that such document qualifies as prior art or constitutes the general knowledge of the skilled person in any jurisdiction. Except in the Examples, or where otherwise explicitly indicated, all numerical quantities in this description specifying amounts of materials, reaction conditions, molecular weights, number of carbon atoms, and the like, are to be understood as modified by the word "about." Unless otherwise indicated, each chemical or composition referred to herein should be interpreted as being a commercial grade material which may contain the isomers, by-products, derivatives, and other such materials which are normally understood to be present in the commercial grade. However, the amount of each chemical component is presented exclusive of any solvent or diluent oil, which may be customarily present

## 18

in the commercial material, unless otherwise indicated. It is to be understood that the upper and lower amount, range, and ratio limits set forth herein may be independently combined. Similarly, the ranges and amounts for each element of the invention can be used together with ranges or amounts for any of the other elements. As used herein, the expression "consisting essentially of" permits the inclusion of substances that do not materially affect the basic and novel characteristics of the composition under consideration.

What is claimed is:

1. A composition comprising:  
an oil of lubricating viscosity; and  
about 0.1 to about 10 weight percent of an N-substituted oxalic acid bisamide or amide-ester containing at least two hydrocarbyl groups of about 12 to about 22 carbon atoms, wherein the N-substituted oxalic acid bisamide or amide-ester comprises an amide-ester represented by the formula:



wherein R<sup>1</sup> and R<sup>2</sup> are independently hydrocarbyl groups of about 12 to about 22 carbon atoms and R<sup>10</sup> is a hydrocarbyl group of 1 to about 22 carbon atoms.

2. The composition of claim 1 further comprising at least one further additive selected from the group consisting of dispersants, detergents, antioxidants, seal swell agents, and anti-wear agents.

3. The composition of claim 1 further comprising at least one additive selected from the group consisting of organic borate esters, organic borate salts, organic phosphorus esters, organic phosphorus salts, inorganic phosphorus acids, and inorganic phosphorus salts.

4. A method for lubricating a transmission, comprising supplying thereto the lubricant of claim 1.

5. A composition comprising:  
an oil of lubricating viscosity; and  
about 0.1 to about 10 weight percent of an N-substituted oxalic acid bisamide or amide-ester containing at least two hydrocarbyl groups of about 12 to about 22 carbon atoms, wherein the N-substituted oxalic acid bisamide or amide-ester comprises a bisamide represented by the formula



wherein R<sup>5</sup> and R<sup>7</sup> are independently a hydrocarbyl group of about 12 to about 22 carbon atoms and R<sup>6</sup> and R<sup>8</sup> are independently hydrogen or a hydrocarbyl group of 10 or fewer carbon atoms or a hydrocarbyl group of about 12 to about 22 carbon atoms.

6. The composition of claim 5 further comprising at least one further additive selected from the group consisting of dispersants, detergents, antioxidants, seal swell agents, and anti-wear agents.

**19**

7. The composition of claim 5 further comprising at least one additive selected from the group consisting of organic borate esters, organic borate salts, organic phosphorus esters, organic phosphorus salts, inorganic phosphorus acids, and inorganic phosphorus salts.

8. A method for lubricating a transmission, comprising supplying thereto the lubricant of claim 5.

9. A composition comprising:  
an oil of lubricating viscosity; and  
about 0.1 to about 10 weight percent of an N-substituted

oxalic acid bisamide or amide-ester containing at least two hydrocarbyl groups of about 12 to about 22 carbon atoms, wherein the N-substituted oxalic acid bisamide or amide-ester comprises an amide-ester represented by the formula:

**20**

wherein R<sup>5</sup> and R<sup>6</sup> are independently hydrocarbyl groups of about 12 to about 22 carbon atoms and R<sup>10</sup> is a hydrocarbyl group of 1 to about 22 carbon atoms.

5

10. The composition of claim 9 further comprising at least one further additive selected from the group consisting of dispersants, detergents, antioxidants, seal swell agents, and anti-wear agents.

15

11. The composition of claim 9 further comprising at least one additive selected from the group consisting of organic borate esters, organic borate salts, organic phosphorus esters, organic phosphorus salts, inorganic phosphorus acids, and inorganic phosphorus salts.

20

12. A method for lubricating a transmission, comprising supplying thereto the lubricant of claim 9.

\* \* \* \* \*